

## UNITED STATES PATENT OFFICE

2,333,821

PHOTOGRAPHING DEVELOPING AND  
FIXING SOLUTION

Martin Salo, Rochester, N. Y., and John W. Mench, West Lafayette, Ind., assignors to Eastman Kodak Company, Rochester, N. Y., a corporation of New Jersey

No Drawing. Application November 25, 1941,  
Serial No. 420,368

## 1 Claim. (Cl. 95—88)

This invention relates to processing solutions for photographic layers of cellulose ethers, containing silver salts in the body of the layer.

Photographic layers of cellulose ether containing about 39 per cent ethoxyl to about 53 per cent ethoxyl containing a light sensitive silver salt, process very slowly in the usual aqueous developing and fixing solutions. We have found that the rate of penetration of aqueous developing and fixing solutions may be considerably increased by diluting standard developing and fixing solutions with certain water miscible organic compounds which have a pronounced swelling action on the cellulose ethers.

It is, therefore, the object of the present invention to provide developing and fixing solutions which permit the dissolved developing or fixing salts to penetrate readily a cellulose ether layer having an alkoxy content of about 39 to 53 per cent.

This object is accomplished by incorporating in a developing or fixing solution a swelling agent for cellulose ether.

The method we use is to take a standard developing or fixing solution and dilute it to the required strength with water and at the same time add to it a sufficient quantity of an organic swelling agent to decrease the time of penetration of the solution. Among the swelling agents which have been found suitable for use in developing and fixing solutions are: methanol, ethanol, propanol, isopropanol, tertiary butanol, ether alcohols such as  $\beta$ -ethoxy ethanol etc. Ketones, such as acetone, are also useful.

The following examples of developing and fixing baths are formulated according to our invention and it is to be understood that they are for the purpose of illustration only.

## EXAMPLE 1

## Developing solution

|                               |        |      |
|-------------------------------|--------|------|
| p-Methyl amino phenol sulfate | grams  | 3.1  |
| Sodium sulfite                | do     | 45.0 |
| Hydroquinone                  | do     | 12.0 |
| Sodium carbonate              | do     | 67.5 |
| Potassium bromide             | do     | 1.9  |
| Water to make                 | liters | 5    |
| Ethyl alcohol                 | grams  | 2762 |

In the preparation of the above solution a liter of a stock developer is diluted as required, for instance, with four volumes of water in processing photographic papers, and then an alcohol is added. The optimum amount of alcohol in the developer depends upon the particular alcohol used,

for example, 45% (by weight) methanol, 35% iso-propanol or ethanol, or 30% n-propanol are satisfactory.

## EXAMPLE 2

## Fixing solution

To a solution of 20 grams of sodium thiosulfate in 80 cc. of water are added 100 grams of methanol. If other alcohols are used instead of methanol, either 63 grams ethanol, 38 grams iso-propanol, or 13 grams n-propanol or tertiary butanol are added in the place of methanol. A ketone such as acetone, in the amount of 45 grams, may also be used with satisfactory results.

The solutions used according to our invention

are of value in treating many types of cellulose ether emulsion, as for instance those containing,

ethyl, propyl and butyl cellulose etc., mixed ethers containing two or more alkoxy groups

such as ethyl propyl or ethyl butyl celluloses,

especially mixed ethers, such as those having a

large share of ethoxyl and a minor proportion of

propoxyl, butyoxyl etc. if such ethers are within

the proper range of etherification so as to be

permeable to the processing solutions of the in-

vention. Thus the cellulose ethyl ethers rang-

ing in alkoxy content from practically com-

pletely etherified ethers to those ethers contain-

ing about 39 per cent alkoxy (less than two

alkoxy groups per  $C_6$  cellulose unit) may be

treated with the solutions of our invention.

Where the degree of etherification is less than

about 39 per cent alkoxy, the layer is more per-

meable to water than the more completely etheri-

fied ethers, and while it may not be necessary

to use the solutions of our invention in process-

ing such layers, the solutions may be used, in

which case the alcohol or ketone content of the

solutions is decreased. Similarly, tests will in-

dicate the proportion of alcohols to be used in

processing emulsion layers of higher ethers or

mixed ethers of cellulose.

In processing cellulose ether layers of about 39 to 53 per cent ethoxyl containing an exposed sil- ver salt, the developing solution of the invention reduces the exposed salt to silver in the region of the exposure. The fixing solution used thereafter removes the unexposed silver salt from the layer.

Other developing and fixing solutions contain- ing the swelling agents of the invention may be used, such as developers containing other develop- ing agents, fog inhibitors, preservatives, etc., and fixing solutions containing other fixing agents, hardeners, etc.

By the term "ethoxyl" as used herein, we mean the alkoxy content of those cellulose ethyl ethers containing only ethoxyl, and of those cellulose ethers containing a major share of ethoxyl and a minor proportion of propoxyl, butoxyl or similar group.

It is to be understood that the disclosure herein is by way of example, and that we consider as included in our invention all modifications and equivalents falling within the scope of the appended claim.

What we claim is:

The method of processing an exposed photo-

graphic emulsion of silver halide dispersed in a cellulose ethyl ether having an ethoxyl content of about 39 percent to about 53 percent, and free of gelatin, which comprises treating said exposed emulsion in turn with developing and fixing baths, at least one of said baths containing a substantial amount of a water-soluble monohydroxy alcohol, said alcohol acting as a swelling agent for the cellulose ether and thereby decreasing the time required to process said cellulose ether emulsion.

MARTIN SALO.  
JOHN W. MENCH.